

## UNITED STATES PATENT OFFICE

CHESTER S. HEATH, OF SOUTH CHARLESTON, WEST VIRGINIA, ASSIGNOR TO ELECTRO METALLURGICAL COMPANY, A CORPORATION OF WEST VIRGINIA

## ANNEALING PROCESS

No Drawing.

Application filed October 12, 1928. Serial No. 312,211.

My invention relates to softening or annealing processes, and particularly to methods for annealing such alloys as are softened by quenching. One of the objects of my invention is to provide a method for the annealing of various alloy compositions, both ferrous and non-ferrous, which is particularly adapted to softening those iron-chromium alloys which are softened by quenching. Another object is the shortening of time for the conduct of the annealing process and still another object is the production of a softer material than is obtainable by previous processes.

Broadly my invention consists in a heating of the alloy object to an elevated temperature, and a rapid quenching therefrom, repeating the cycle of heating and quenching a number of times in succession, the alloy being brought to substantially the same temperature in all the heating steps, and being quenched substantially at once upon obtaining the proper heat in each of said heating steps. I believe I am the first to discover that a greater annealing and softening is obtainable in an alloy of any kind, and particularly in a chrome-iron alloy, by a repeated heating and quenching of the material from an elevated temperature.

The following tests and experiments indicate the objects of my invention, the character of my process, and the results obtained by it.

A well-known, corrosion-resistant, chromium alloy, having the following composition, was used as material for demonstrating the effect of my process of the application of repeated cycles of heating and quenching thereto.

|             |           |
|-------------|-----------|
| 40 Chromium | 27.77%    |
| Carbon      | 0.25%     |
| Nickel      | 0.25%     |
| Silicon     | 0.12%     |
| Manganese   | 0.33%     |
| 45 Iron     | Remainder |

This material was rolled to 20 gauge sheet, with care to conduct the rolling at a high temperature. The material was tested in the condition "as rolled", and also after various heat treatments, including that of my new process, with the results indicated in the appended table:

| Expt. No. | Heat treatment                                                                                             | Number of samples treated | Average Erichsen value |
|-----------|------------------------------------------------------------------------------------------------------------|---------------------------|------------------------|
| 8         | As rolled                                                                                                  | 5                         | 65                     |
| 3         | Heated at 900° C. for 12 hrs. and quenched in water                                                        | 5                         | 3.25                   |
| 1         | Heated 10 times to temperatures between 900 and 1000° C. and quenched in water between successive heatings | 5                         | 70                     |

It may be noted that the material as rolled has a low Erichsen value. It may be further noted that a heating to 900° C. for a long period of time such as 12 hours and then quenching in water, the best prior practice, results in a substantial softening, as indicated by the higher Erichsen value. It may be further noted that 10 cycles of heating to temperatures at or slightly above 900° C. and quenching at once in water, which series of operations may be conducted in an elapsed time of about an hour and a half for the 10 cycles, produces a still higher Erichsen value, showing a gain in softness and a very substantial saving in the time required for the annealing operation. That is to say, the total time required for the process of the invention is materially less than that required to secure the same degree of softening of like material by the old methods which consisted of a single quench preceded by a sustained heating of the material.

On another sample of commercial iron-chromium alloy having high corrosion-resistance, and containing 25.4% of chromium, and 0.17% of carbon, the process of my in-

vention produced equally good results, as shown by the following table.

| Expt. No. | Heat treatment                                                 | Yield point | Ultimate strength | % Elongation in 2" | % red. area |
|-----------|----------------------------------------------------------------|-------------|-------------------|--------------------|-------------|
| 1.        | As Rec'd.                                                      | 68800       | 86250             | 23.5               | 47.2        |
| 2.        | do                                                             | 68800       | 86300             | 26.0               | 52.2        |
| 3.        | 850° C.—16 hrs. Quenched in water once                         | 55600       | 77800             | 31.0               | 61.6        |
| 10 12.    | 850°—900° C.—35 mins. Alternately heated and quenched 5 times  | 50900       | 76300             | 32.0               | 69.3        |
| 5.        | 800°—900° C.—Alternately heated and quenched in water 10 times | 53600       | 78700             | 32.0               | 62.7        |
| 6.        | 800°—900° C.—Alternately heated and quenched in water 20 times | 52150       | 75900             | 35.0               | 65.3        |

It may be noted from this table that substantial gains in softness, as indicated by the measurements of the elongation, and the reduction in area, are obtainable by the process of my invention and that the gains are progressive with increase in the number of cycles of heating and quenching through which the material is put.

25 It may be noted that the temperature to, or above, which the material should be heated varies somewhat with the composition of the alloy. The desirable temperature will usually not be below 700° C. or 800° C. I find, however, that if the heating is conducted to a temperature between about 800° C. to 1000° C. a sufficiently high temperature is obtained to be suitable for substantially all of the chromium containing alloys. It may be noted that in some cases it is undesirable to heat the materials to a temperature much above 1000° C. since at a temperature of 1050° C. to 1250° C. a rapid coarsening of the grain of some of the alloys occurs, which may detract from some of the desirable properties of the material. The above observations apply to the majority of the iron chromium alloys. When the process of my invention is applied to non-ferrous alloys, the desirable temperature may depart considerably from those above indicated, depending upon the character and composition of the alloys treated.

50 The process of my invention is applicable to other alloys than the simple chrome-iron alloys above discussed. It may be applied to alloys of other compositions, especially of those containing nickel, for the production of equally advantageous results. I find that 55 a chrome-nickel-iron alloy having the following composition is softened rapidly, easily and thoroughly by the same treatment.

|           |           |
|-----------|-----------|
| Chromium  | 19.20%    |
| Nickel    | 8.44%     |
| Silicon   | 0.43%     |
| Manganese | 0.23%     |
| Carbon    | 0.14%     |
| Iron      | Remainder |

55 Samples of the above alloy were rolled to

20 gauge sheet, at a suitably elevated temperature, and specimens suitable for Erichsen test were cut from the rolled sheet. The samples were heat treated as indicated in the following table with the indicated results. 70

| Expt. No. | Heat treatment                                                        | Number of samples tested | Average Erichsen value |
|-----------|-----------------------------------------------------------------------|--------------------------|------------------------|
| 1.        | As rolled.                                                            | 5                        | 7.2                    |
| 4.        | Heated at 900° C. for 15 hrs, and quenched in water.                  | 5                        | 7.8                    |
| 2.        | Heated 10 times between 900 and 1000° C. and quenched in water.       | 4                        | 8.3                    |
| 6.        | Heated at 1050° C. for 1 hr, and quenched in water.                   | 5                        | 8.6                    |
| 8.        | Heated 10 times to 1050° C. and quenched in water after each heating. | 5                        | 8.7                    |
| 9.        | Heated at 1100° C. for 1 hr. and quenched in water.                   | 5                        | 8.5                    |
| 11.       | Heated 10 times at 1100° C. and quenched in water after each heating. | 5                        | 8.8                    |
| 12.       | Heated at 1150° C. for 1 hr. and quenched in water.                   | 5                        | 7.8                    |
| 14.       | Heated 10 times to 1150° C. and quenched in water after each heating. | 5                        | 9.2                    |

It may be noted that 10 cycles of heating to 900° C., and quenching at once in water, gives a greater softening than a heating to 900° for 15 hours and thereafter quenching with water. Thus, not only is the material more completely softened, but the softening is obtained more conveniently. It is thus evident that this alloy as well can be advantageously softened by the process of my invention. 90

The process of my invention is not only applicable to those iron-chromium alloys which are softened by quenching, but is also applicable to non-ferrous alloys. Alloys containing nickel, manganese, and copper have been found to have very valuable physical and electrical properties. Only a few however of the possible alloys of these three materials are sufficiently ductile as cast to be workable in the cold. (The range of ductile alloys is shown by ternary diagrams by Pilling, "Some electrical properties of copper-nickel-manganese alloys", in the Transactions of the American Electrochemical Society, 1925.) 100

105 In order to determine the effect of the process of my invention upon non-ferrous alloys, and particularly upon the alloys of this type which are found to be difficult to work, it was applied to an alloy having the following composition: 110

| NI    | Mn    | Cu    |
|-------|-------|-------|
| 51.25 | 27.44 | 20.50 |

115 This alloy is known to have valuable properties, but is found to be so difficult to work that it is unused. The alloy material was cast into one half inch square bars, and forged at 900° C. into flat specimens having a thickness of  $\frac{1}{16}$  of an inch, about  $\frac{3}{4}$  of an inch wide and three inches long. Various of these 120

specimens were then given the treatments outlined in the following table:

| 5  | Bend specimen | Heat treatment                                            | Fiber elongation | Per cent |
|----|---------------|-----------------------------------------------------------|------------------|----------|
|    | #1            | As forged                                                 |                  | 9        |
| 10 | #2            | Heated for seven minutes 900° C. and water quenched       |                  | 15       |
|    | #4            | Heated to 900° C. for 1 hour. Water quenched              |                  | 19       |
|    | #3            | Heated to 900° C. for 5 hours. Water quenched             |                  | 17       |
|    | #3            | Alternately heated to 900° C. and water quenched 10 times |                  | 34       |

After the respective treatments, the various samples were machined upon opposite sides and bent to obtain the fiber elongations, which are recorded in the above table. It will be observed that the application of the annealing process of my invention to this material results in a conspicuous gain in efficiency of annealing.

By the process of my invention I am thus enabled to obtain a greater softness in various brittle alloys, both ferrous and non-ferrous, than is obtainable by other processes, and in many cases in a much shorter period of time than is required for other, less effective, annealing processes. My invention thus simplifies and cheapens the fabrication of articles made from such alloys and may make commercially usable certain alloys which are otherwise too brittle to be used.

While I have disclosed but a limited number of embodiments of my invention, it is capable of still other modifications therefrom without departure from the spirit thereof and it is desired therefore that only such limitations shall be imposed upon the appended claims as are stated therein or required by the prior art.

40 I claim as my invention:

1. The process of treating an alloy which is initially in a hard state, and which alloy is adapted, by its composition, to be softened by bringing it to a high temperature and then quenching it; which process comprises heating the alloy to and quenching it from a temperature adapted to give substantially the maximum softening effect which can be obtained by a single quench; and then repeating the heating and quenching several times, the alloy being brought to substantially the same temperature in all the heating steps; the total time required for said process being materially less than that required to secure the same degree of softening of like material by a single quench preceded by a sustained heating of said material at said temperature.

2. The process of treating an iron-chromium alloy which is initially in a hard state, and which alloy is adapted, by its composition, to be softened by bringing it to a high temperature and then quenching it; which process comprises heating the alloy to and quenching it from a temperature adapted to give substantially the maximum softening effect

which can be obtained by a single quench; and then repeating the heating and quenching several times, the alloy being brought to substantially the same temperature in all the heating steps; the total time required for said process being materially less than that required to secure the same degree of softening of like material by a single quench preceded by a sustained heating of said material at said temperature.

3. The process of treating an alloy which is initially in a hard state, and which alloy is adapted, by its composition, to be softened by bringing it to a high temperature and then quenching it; which process comprises heating the alloy to and quenching it from a temperature adapted to give the maximum softening effect which can be obtained by a single quench; and then repeating the heating and quenching several times, the alloy being brought to substantially the same temperature in all the heating steps, and the said alloy being quenched substantially at once upon obtaining the proper heat in each of said heating steps.

4. The process of treating an iron-chromium alloy which is initially in a hard state, and which alloy is adapted, by its composition, to be softened by bringing it to a high temperature and then quenching it; which process comprises heating the alloy to and quenching it from a temperature between about 800° C. and 1000° C., and then repeating the heating and quenching several times, the alloy being brought to substantially the same temperature in all the heating steps, and the said alloy being quenched substantially at once upon obtaining the proper heat in each of said heating steps.

5. The process of treating a nickel-manganese-copper alloy which is initially in a hard state, and which alloy is adapted, by its composition, to be softened by bringing it to a high temperature and then quenching it; which process comprises heating the alloy to and quenching it from a temperature adapted to give the maximum softening effect which can be obtained by a single quench; and then repeating the heating and quenching several times, the alloy being brought to substantially the same temperature in all of the heating steps; the total time required for said process being materially less than that required to secure the same degree of softening of said alloy by a single quench preceded by a sustained heating of said material at said temperature.

In testimony whereof, I affix my signature.  
CHESTER S. HEATH.

125

130